

## UNITED STATES PATENT OFFICE.

JAMES H. GRAVELL, OF ELKINS PARK, PENNSYLVANIA.

## COMPOSITION OF MATTER AND PROCESS FOR PREPARING METAL FOR PAINTING.

No Drawing.

Application filed October 11, 1923. Serial No. 667,822.

*To all whom it may concern:*

Be it known that I, JAMES H. GRAVELL, a citizen of the United States, residing at Elkins Park, in the county of Montgomery and State of Pennsylvania, have invented a new and useful Composition of Matter and Process for Preparing Metal for Painting, of which the following is a specification.

This invention relates to improvements in

10 the art of preparing for painting metal generally and specifically metal that is liable to rust during fabrication processes, such for instance as cold rolled steel used in the manufacture of automobile bodies.

One object of the invention is to remove from the metal oil, rust, dirt, hand-marks, acid runs, soldering fluids and the like so that the metal may be properly prepared to receive a coating of paint, varnish or 20 similar material. As material to which my invention relates is usually applied by the hands, a further object of the invention is to provide a material, which when properly manipulated, is not harmful to the skin.

25 It has been the custom to use mixtures of phosphoric acid containing higher alcohols, such as butyl alcohol, but owing to the great oil solvent properties of those alcohols the natural oil of the skin is removed and the 30 hands are no longer protected against the danger of chapping. I have discovered that acetates of the lower alcohols, such as ethyl acetate, can be used to advantage in connection with mixtures containing metal 35 etching acids to make them properly wet the surface to be cleaned and to avoid their unduly attacking the hands.

Since metal etching acids and ethyl acetate are not miscible, it is necessary to 40 add alcohol and one of the lower alcohols (ethyl, methyl, or propyl) may be added in order to make them miscible. Water must also be added to bring the mixture to the proper commercial strength. However, an 45 admixture of ethyl acetate, alcohol, and water is not stable, but on standing a certain amount of acetic acid is formed at the expense of the ethyl acetate and water; therefore in order to stabilize the admixture I 50 provide acetic acid which not only accomplishes that result but also assists the metal etching acid in cleaning the work.

By experiment I have discovered that it is necessary to have in a stabilized admixture of metal etching acid, water and acetic acid at least 7% by volume of ethyl acetate and at least 30% by volume of alcohol in order to properly perform the work of causing the acid or acids to wet an oily surface. This can be accomplished by using commercial materials according to the following formula:

## Formula No. 1.

|                                       | Gallons. |
|---------------------------------------|----------|
| 85% ortho phosphoric acid             | 0.124    |
| Alcohol (ethyl, methyl or --- propyl) | .368     |
| Ethyl acetate                         | .082     |
| 80% acetic acid                       | .068     |
| Water                                 | .358     |
|                                       | 70       |

Owing to the presence of the acetic acid the above admixture is primarily stable.

It is possible to omit either the ethyl acetate or the acetic acid by proportioning the other ingredients in such a way that when the admixture has by reaction and combination become stabilized, the missing ingredient will be formed and be present in the resulting stabilized admixture. For instance the following formula may be used 75 which after standing becomes practically the same as formula No. 1.

## Formula No. 2.

|                           | Gallons. |
|---------------------------|----------|
| 85% ortho phosphoric acid | 0.124    |
| Alcohol                   | .300     |
| Ethyl acetate             | .150     |
| Water                     | .426     |

As a result of standing the ethyl acetate 90 and the water decrease, acetic acid forms and the alcohol increases.

If desired the ethyl acetate may be replaced by acetic acid provided the remaining ingredients are properly proportioned 95 as shown in

## Formula No. 3.

|                           | Gallons. |
|---------------------------|----------|
| 85% ortho phosphoric acid | 0.124    |
| Alcohol                   | .450     |
| Acetic acid 80%           | .150     |
| Water                     | .276     |

In becoming stabilized or balanced, on

standing, this formula becomes practically the same as formula No. 1.

The above formulas may be altered to a great extent provided the minimum of ethyl acetate and alcohol is maintained, without departing from the spirit of the invention, for instance, the phosphoric acid may be replaced by sulphuric acid or hydrochloric acid in various amounts, or additions of metallic salts or acid salts may be made, or acid salts may be used instead of acids. However, in preparing steel for painting, phosphoric acid is preferably present because it greatly assists in preventing the metal from rusting after the admixture has been used.

A very practical formula embodying the above suggested variation is:

20 *Formula No. 4.*

|                           |            |
|---------------------------|------------|
| 85% ortho phosphoric acid | 0.124 gal. |
| Denatured alcohol         | .300 "     |
| Ethyl acetate             | .150 "     |
| Sodium acid sulphate      | .700 lbs.  |
| Water                     | .396 gal.  |

According to my process the work just prior to painting is treated with a balanced alcohol-ethyl acetate-acetic acid-water admixture in the presence of a metal etching acid by spraying, dipping or brushing. If necessary, the action of the admixture may be assisted by an abrasive. When the metal has been sufficiently cleaned, the spent admixture is removed. This may be done by wiping, by blowing off for instance with air or steam, or by washing with water. After the spent admixture has been completely removed and the surface has become dry, it is ready for painting.

From the foregoing description it appears that I have provided a composition of matter for cleaning metal surfaces in which the proportion of the ingredients is fixed and stable, and which can be at all times relied upon to contain at least the necessary minimum quantities of alcohol and acetate, and from the foregoing description it further appears that by providing ethyl acetate I can avoid such use of higher alcohols, for example, butyl alcohol, as might result in undue attacks upon the hands of the workmen.

55 I claim:

1. A composition of matter for preparing metal for painting comprising an admixture of a metal etching acid and a stable solution containing alcohol, ethyl acetate and water.

2. A stable composition of matter for preparing metal for painting containing a metal etching acid and ethyl acetate.

3. A stable composition of matter for preparing metal for painting containing a

metal etching acid, ethyl acetate and alcohol.

4. A stable composition of matter for preparing metal for painting containing a metal etching acid, ethyl acetate, alcohol 70 and acetic acid.

5. A stable composition of matter for preparing metal for painting containing a metal etching acid, ethyl acetate, alcohol, 75 acetic acid and water.

6. A stable composition of matter for preparing metal for painting containing a metal etching acid and at least 7% by volume of ethyl acetate and at least 30% by volume of alcohol. 80

7. A stable composition of matter for preparing metal for painting containing phosphoric acid and ethyl acetate.

8. A stable composition of matter for preparing metal for painting containing phosphoric acid, ethyl acetate and alcohol. 85

9. A stable composition of matter for preparing metal for painting containing phosphoric acid, ethyl acetate, alcohol and water. 90

10. A stable composition of matter for preparing metal for painting containing phosphoric acid, ethyl acetate, alcohol, water and acetic acid.

11. A stable composition of matter for preparing metal for painting containing phosphoric acid, ethyl acetate, alcohol, water, acetic acid and a soluble acid sulphate. 95

12. A stable composition of matter for preparing metal for painting containing phosphoric acid, ethyl acetate, alcohol, water, acetic acid and sodium acid sulphate. 100

13. The method of preparing metal for painting consisting in treating it with a metal etching acid in the presence of a stabilized solution of ethyl acetate. 105

14. The method of preparing metal for painting consisting in treating it with phosphoric acid in the presence of a stabilized 110 solution of ethyl acetate.

15. The method of preparing metal for painting consisting in treating it with phosphoric acid in the presence of a stabilized 115 admixture of ethyl acetate, alcohol, water and acetic acid.

16. The method of preparing metal for painting consisting in treating it with phosphoric acid in the presence of a stabilized 120 admixture of ethyl acetate, alcohol, water and acetic acid, removing the said acid and admixture and causing or permitting the metal to dry.

17. A composition of matter for preparing metal for painting comprising a stable 125 fluid admixture of metal etching acid, water, a lower alcohol, ethyl-acetate, and acetic acid, the alcohol and ethyl-acetate content being primarily fixed by the pres- 130

ence of acetic acid which opposes acetic acid-forming reaction between the alcohol and ethyl acetate.

18. A composition of matter for preparing metal for painting comprising a stable fluid admixture of phosphoric acid, water, a lower alcohol, ethyl-acetate, and acetic

acid, the alcohol and ethyl-acetate content being primarily fixed by the presence of acetic acid which opposes acetic acid-forming reaction between the alcohol and ethyl acetate. <sup>10</sup>

JAMES H. GRAVELL.